

## UNITED STATES PATENT OFFICE

2,481,205

SIMULTANEOUSLY SCOURING AND  
BLEACHING WOOL

Archie Louis Dubeau, Rumford, R. I., assignor to  
Mathieson Chemical Corporation, a corpora-  
tion of Virginia

No Drawing. Application April 19, 1946,  
Serial No. 663,636

3 Claims. (Cl. 8—139)

1

This invention relates to improvements in the processing of wool including both shorn wool and "pulled" wool.

In accordance with conventional practice, wool before utilization in the production of yarn is subjected to treatment in a series or train of five treating vessels known as "bowls." In the first bowl of the train, the wool is desuited by washing with cold water. In the 2nd and 3rd bowls, the desuited wool is scoured, usually at a temperature of about 125° F., with an aqueous solution of soap and sodium carbonate. The 4th and 5th bowls are essentially rinsing bowls, but the last bowl, from which the wool is passed to a dryer, may contain a bleaching agent, conventionally hydrogen peroxide.

The scouring in the No. 2 and No. 3 bowls, when the system does not include mechanical grease recovery equipment, proceeds with periodic removal of about half of the solution and replacement of the removed portion with warm water, fresh soda ash and soap being added to maintain the solution at the desired chemical concentration. Soda ash and soap are also continuously or intermittently added during the periods between the half dumps. At the end of 24 hours, the bowls are usually completely emptied, thoroughly washed and charged with fresh liquor.

Where continuous grease recovery equipment is employed, the scouring solution is circulated through the wool and through the grease machine, the solution ordinarily being caused to flow from the No. 3 bowl to the No. 2 bowl, through the grease machine and then back to the No. 3 bowl. Some operators, however, prefer to recover the grease from the No. 2 bowl only, in which case the scouring liquid is withdrawn from the wool exit end of the No. 2 bowl, passed through the grease machine, then returned to the No. 2 bowl at the wool entering end of the bowl. In either case the scouring liquor is periodically fortified by the addition of fresh chemicals.

If during the scouring of shorn wool by the conventional method, a sample of the scouring liquor is taken from the first bowl, in which about 90% of the scouring is accomplished, before each addition of soda ash and a double titration with .09 normal HCl run on the samples using phenolphthalein as the indicator in the first titration and methyl orange as the indicator in the second, it will be found that the spread between the phenolphthalein end point and the methyl orange end point (total alkalinity) in terms of cubic centimeters of acid becomes progressively greater. This means that the proportion of carbonate con-

verted to bicarbonate during the operation progressively increases, albeit a part of the total alkalinity may be due to the presence of compounds other than sodium carbonate and sodium bicarbonate.

The accompanying Table 1, submitted in illustration of the immediate foregoing, is based on an operation carried out without the use of mechanical grease recovery equipment in which the wool was treated at the rate of about 1000 pounds per hour. The liquor in the No. 2 bowl consisted initially of 3500 gallons of water, 120 gallons of soda ash solution containing 92.5 pounds of soda ash, and 30 gallons of soap solution containing 8.3 pounds of soap, while the liquor in the No. 3 bowl at the beginning of the operation consisted of 1500 gallons of water, 60 gallons of soda ash solution containing 46.25 pounds of soda ash, and 30 gallons of soap solution having a soap concentration of 0.277 pounds per gallon. As the scouring proceeded, the liquor was fortified every 45 minutes by adding 36 gallons of soda ash solution containing 27.8 pounds of soda ash to the No. 2 bowl and by adding 18 gallons of soda ash solution containing 13.9 pounds of soda ash together with 12 gallons of soap solution containing 3.33 pounds of soap to the No. 3 bowl. At the end of each six hour period, half of the scouring solution was withdrawn from both scouring bowls and the withdrawn solution replaced with water. Following each addition of make-up water, 90 gallons of soda ash solution containing 69.5 pounds of soda ash and 30 gallons of soap solution containing 0.277 pounds of soap per gallon were added to the No. 2 bowl, and 45 gallons of soda ash solution containing 34.6 pounds of soda ash and 30 gallons of soap solution were added to the No. 3 bowl.

TABLE I

| Sample No. | C. c.'s .09 normal HCl to Phenolphthalein End Point | Total c. c.'s .09 normal HCl to Methyl Orange End Point | Alkalinity Calculated as $\text{Na}_2\text{CO}_3$ and $\text{NaHCO}_3$ | Apparent Ratio, Carbonate: Bicarbonate |
|------------|-----------------------------------------------------|---------------------------------------------------------|------------------------------------------------------------------------|----------------------------------------|
| 1.....     | 2                                                   | 5.3                                                     | 2.12 1.09                                                              | 1:0.51                                 |
| 2.....     | 1.9                                                 | 6.9                                                     | 2.01 2.6                                                               | 1:1.20                                 |
| 3.....     | 2.3                                                 | 8.6                                                     | 2.44 3.36                                                              | 1:1.39                                 |
| 4.....     | 2.3                                                 | 10.6                                                    | 2.44 5.04                                                              | 1:2.06                                 |
| 5.....     | 2.4                                                 | 13.1                                                    | 2.54 7.17                                                              | 1:2.82                                 |
| 6.....     | 2.9                                                 | 14.6                                                    | 3.07 7.59                                                              | 1:2.47                                 |
| 7.....     | 2.9                                                 | 16.1                                                    | 3.07 8.65                                                              | 1:2.82                                 |
| 8.....     | 2.7                                                 | 16.7                                                    | 2.86 9.49                                                              | 1:3.32                                 |
| 9.....     | 2.4                                                 | 17.3                                                    | 2.54 10.5                                                              | 1:4.13                                 |

The samples in the table were taken immediately before each addition of soda ash and soap. Although the total alkalinity is calculated as due entirely to sodium carbonate and bi-

carbonate, it is to be understood that a relatively small part of the alkalinity may derive from other compounds formed during the scouring having a pH value similar to that of sodium bicarbonate. Alkalinity as sodium carbonate is calculated by multiplying the cubic centimeters of acid to the phenolphthalein end point by 1.06; alkalinity as sodium bicarbonate by subtracting twice the cubic centimeters of acid to the phenolphthalein end point from the cubic centimeters of acid to the methyl orange end point and multiplying the difference by 0.84. The table shows that in the conventional process, in which no effort is made to control the carbonate: bicarbonate ratio, the weight of bicarbonate present in the solution soon exceeds twice the weight of carbonate present.

In accordance with the present invention I include sodium chlorite as a component of the scouring liquor and I so control the composition of the liquor that the ratio of the figure obtained by multiplying the cubic centimeters of .09 normal HCl required to reach the phenolphthalein end point by 1.06 to the figure obtained by multiplying the difference between twice the cubic centimeters of .09 normal HCl to phenolphthalein end point and the cubic centimeters of .09 normal HCl required to reach the methyl orange end point by 0.84 is kept substantially at all times within the range of about 1:0.5 to 1:2. With the inclusion of the chlorite, bleaching as well as scouring of the wool is achieved.

It will be understood that reference in the appended claims to the weight ratio of apparent carbonate to bicarbonate is intended to mean the ratio determined by the procedure just described.

Though the bleaching of wool with hydrogen peroxide solutions has been practiced extensively as indicated in the forepart hereof, hydrogen peroxide solutions have not been entirely satisfactory for the reason that they tend to make the wool harsh. Highly concentrated solutions have been known to materially damage the wool. At the lower concentrations the bleaching action of hydrogen peroxide is objectionably slow.

According to the present invention whereby simultaneous scouring and bleaching is achieved, the quality of the wool is in no way reduced, in fact the treated wool is almost invariably less harsh than wool processed by the conventional method without peroxide.

I have obtained excellent results using the sodium chlorite in concentrations as low as 0.01% and as high as about 2% by weight of available chlorine. Still higher concentrations of the chlorite may be used without danger of damaging the wool, but without materially improved results. Generally satisfactory results are obtained by the use of the chlorite in concentrations of about 0.02-0.03% based on the weight of available chlorine.

The chlorite may be employed in only one of the scouring bowls in the previously described train or it may be used in both bowls. The fourth or rinsing bowl of the train may or may not contain chlorite. No adjustment of temperature is required on account of the chlorite, i. e. the conventional temperatures may be used.

That the chlorite would be effective in the environment of my process is surprising. Although use of chlorites in the bleaching of cellulosic material has previously been proposed, in that application it is necessary either to activate the chlorite, as with chlorine or a hypochlorite, or to employ the chlorite in an acid medium. Any

attempt to use a chlorite in the bleaching of wool has heretofore been discouraged by the fact that the desired characteristics of wool are destroyed or are at least adversely affected by treatment with chlorine or with chlorine compounds, such as the hypochlorites which in use evolve chlorine.

In the scouring of shorn or other acidic wools, the composition of the scouring liquor can be maintained within the prescribed limits on alkalinity, with advantage, through the continuous or intermittent introduction of controlled amounts of aqueous caustic soda. Less preferably, aqueous caustic potash or an aqueous solution of an alkaline earth metal hydroxide, such as calcium hydroxide may be introduced into the liquor. The added alkali, it will be understood, acts to convert excess bicarbonate back to carbonate in accordance with the equation:



The alkaline solution is not, of course, added from the very beginning of the scouring when the concentration of bicarbonate is negligible, in fact, it is advantageous in preparing the initial solution to add bicarbonate:

In the case of "pulled" wool where sodium bicarbonate is not formed as an incident of the scouring, the wool being alkaline from pre-treatment with lime, the desired composition of the scouring liquor is maintained in accordance with my invention by the continuous or intermittent addition of sodium bicarbonate or an acid or acid salt, such as acid phosphate. The initial solution in the instance of alkaline wools should be made up to contain bicarbonate in an amount indicated by the limits above.

In a preferred embodiment of my invention as applied to acid wool, the caustic solution is added to the first scouring bowl only, and in the company of liquor removed from the bowl rather than directly to the bowl. The caustic may become completely reacted before it enters the bowl. Direct addition of the caustic solution to the bowl appears disadvantageous as resulting in localized harshening of the wool. The liquor to which the caustic solution is to be added is preferably withdrawn from the wool exit end of the bowl, passed through a trough or tank where the caustic solution is charged to the liquor, and the adjusted liquor pumped back into the wool-entering end of the bowl. The caustic solution most suitably has a NaOH concentration of about 1.5 pounds per gallon. Where the caustic is added continuously, which is preferable in most cases, a variable feed proportioning pump may be employed with advantage. The rate at which the caustic solution is added is determined, as previously indicated, by the rate of bicarbonate formation.

The practice of my invention is further illustrated by the following examples:

#### Example 1

The wool treated is shorn wool. The run is started immediately after the bowls had been half-emptied and the removed scouring liquor replaced with water. Upon titration of 10 c. c. samples, following addition of make-up chemicals, including chlorite, with .09 normal HCl, 2.7 c. c. of acid is required to reach the phenolphthalein end point and 7.1 c. c. of acid is required to reach the methyl orange end point.

The wool is fed to the system at the rate of about 1200 pounds per hour. The caustic solu-

tion used consists of about 20 pounds sodium hydroxide in 50 gallons of water. The solution is continuously added to liquor from the first scouring bowl only, and at a rate equivalent to 3.5 pounds of NaOH per thousand pounds of wool. Data on typical runs are given in accompanying Tables 2 and 3:

My process as compared with the conventional method is definitely cheaper in both chemical and labor costs. Because the wool can be charged at a constant high rate and because less changing of the liquor is required, greatly increased production can be achieved with same equipment. In many instances, the process can be

TABLE II

| Time  | Sample No. | C. c.'s .09 normal HCl to end point Phenolphthalein | C. c.'s .09 normal HCl to end point Methyl Orange | Chlorite Concentration (based on weight of available chlorine) | Alkalinity Calculated as $\text{Na}_2\text{CO}_3$ and $\text{NaHCO}_3$ | Apparent Ratio, Carbonate:Bicarbonate |
|-------|------------|-----------------------------------------------------|---------------------------------------------------|----------------------------------------------------------------|------------------------------------------------------------------------|---------------------------------------|
| 11.30 | 1          | 3.4                                                 | 10.5                                              | .014                                                           | 3.60                                                                   | 3.11                                  |
| 12.00 | 2          | 3.1                                                 | 10.5                                              | .016                                                           | 3.29                                                                   | 3.61                                  |
| 12.30 | 3          | 3.3                                                 | 10.5                                              | .006                                                           | 3.5                                                                    | 3.28                                  |
| 1.00  | 4          | 3.0                                                 | 10.5                                              | .034                                                           | 3.18                                                                   | 3.78                                  |
| 1.30  | 5          | 2.9                                                 | 10.7                                              | .034                                                           | 3.07                                                                   | 4.11                                  |
| 2.00  | 6          | 2.7                                                 | 11.2                                              | .009                                                           | 2.86                                                                   | 4.89                                  |
| 2.30  | 7          | 2.6                                                 | 9.7                                               | .025                                                           | 2.76                                                                   | 3.78                                  |
| 3.00  | 8          | 2.4                                                 | 9.7                                               | .019                                                           | 2.54                                                                   | 4.11                                  |
| 3.30  | 9          | 2.4                                                 | 10.2                                              | .008                                                           | 2.54                                                                   | 4.53                                  |
| 4.00  | 10         | 2.5                                                 | 10.2                                              | .028                                                           | 2.65                                                                   | 4.37                                  |
| 4.30  | 11         | 2.6                                                 | 10.3                                              | .026                                                           | 2.76                                                                   | 4.28                                  |
| 5.00  | 12         | 2.6                                                 | 11.2                                              | .023                                                           | 2.76                                                                   | 5.04                                  |

TABLE III

| Time  | Sample No. | C. c.'s .09 normal HCl to end point Phenolphthalein | C. c.'s .09 normal HCl to end point Methyl Orange | Chlorite Concentration (based on weight of available chlorine) | Alkalinity Calculated as $\text{Na}_2\text{CO}_3$ and $\text{NaHCO}_3$ | Apparent Ratio Carbonate:Bicarbonate |
|-------|------------|-----------------------------------------------------|---------------------------------------------------|----------------------------------------------------------------|------------------------------------------------------------------------|--------------------------------------|
| 9.30  | 1          | 3.7                                                 | 11.3                                              | .043                                                           | 3.92                                                                   | 3.28                                 |
| 10.00 | 2          | 3.9                                                 | 12.6                                              | .055                                                           | 4.13                                                                   | 4.05                                 |
| 10.30 | 3          | 4.1                                                 | 13.2                                              | .042                                                           | 4.35                                                                   | 4.2                                  |
| 11.00 | 4          | 4.7                                                 | 13.9                                              | .048                                                           | 4.98                                                                   | 3.78                                 |
| 11.30 | 5          | 3.9                                                 | 13.1                                              | .036                                                           | 4.13                                                                   | 4.45                                 |
| 12.00 | 6          | 4.3                                                 | 13.3                                              | .051                                                           | 4.56                                                                   | 3.85                                 |
| 12.30 | 7          | 4.0                                                 | 13.3                                              | .047                                                           | 4.24                                                                   | 4.45                                 |
| 1.00  | 8          | 4.0                                                 | 13.4                                              | .038                                                           | 4.24                                                                   | 4.63                                 |
| 1.30  | 9          | 3.8                                                 | 13.0                                              | .052                                                           | 4.02                                                                   | 4.53                                 |
| 2.00  | 10         | 3.4                                                 | 12.8                                              | .063                                                           | 3.60                                                                   | 5.04                                 |
| 2.30  | 11         | 3.4                                                 | 12.8                                              | .064                                                           | 3.60                                                                   | 5.04                                 |
| 3.00  | 12         | 3.2                                                 | 12.8                                              | .054                                                           | 3.39                                                                   | 5.38                                 |
| 3.30  | 13         | 3.4                                                 | 12.6                                              | .059                                                           | 3.60                                                                   | 4.89                                 |
| 4.00  | 14         | 3.1                                                 | 12.8                                              | .055                                                           | 3.29                                                                   | 5.64                                 |
| 4.30  | 15         | 3.2                                                 | 13.0                                              | .060                                                           | 3.39                                                                   | 5.64                                 |

## Example 2

"Pulled" wool is treated at the rate of 700 pounds per hour using conventional bowls. The treatment is carried out at a temperature of 130° F. and the make-up on the scouring bowls is as follows:

Water \_\_\_\_\_ gallons 3,750  
 Sodium bicarbonate \_\_\_\_\_ pounds 300  
 Sodium carbonate \_\_\_\_\_ do 180  
 Soap \_\_\_\_\_ do 12  
 Sodium chlorite \_\_\_\_\_ do 10

During the course of the run, 100 pounds additional of sodium bicarbonate is added to the first scouring bowl in increments of about 16 pounds. Data on such a run is given in the following table:

TABLE IV

| Time  | pH  | $\text{ClO}_2$ Conc. <sup>1</sup> | Per Cent $\text{Na}_2\text{CO}_3$ | Per Cent $\text{NaHCO}_3$ | Ratio $\text{Na}_2\text{CO}_3:\text{NaHCO}_3$ |
|-------|-----|-----------------------------------|-----------------------------------|---------------------------|-----------------------------------------------|
| 2.30  | 9.1 | .035                              | .3                                | .5                        | 1:1.7                                         |
| 4.00  | 9.5 | .030                              | .54                               | .61                       | 1:1.14                                        |
| 6.00  | 9.7 | .028                              | .72                               | .55                       | 1:1.16                                        |
| 7.15  | 9.8 | .032                              | .76                               | .43                       | 1:1.56                                        |
| 9.30  | 9.8 | .031                              | .74                               | .53                       | 1:1.71                                        |
| 11.00 | 9.8 | .027                              | .76                               | .45                       | 1:1.59                                        |

<sup>1</sup> Based on weight of available chlorine.

45 operated to increase production more than 100%, say from 300 pounds of wool per hour to 600-700 pounds per hour and with noticeable improvement in the quality of the processed wool.

50 The bleaching action of the chlorite in my process appears to be enhanced by its environment and conversely the presence of the chlorite in the liquor seems to increase the scouring ability of the liquor. At the pH at which the liquor is maintained according to the invention, little, if any, chlorine dioxide is evolved which is distinctly advantageous because of the corrosive properties of this gas.

55 I claim:

60 1. A continuous process for simultaneously scouring and bleaching wool which comprises continuously passing the wool to be treated in contact with an aqueous liquor containing soda ash, sodium bicarbonate, soap and sodium chlorite and maintaining the composition of the liquor such that the weight ratio of apparent carbonate to bicarbonate is within the range of 1:0.5 to 1:2 substantially throughout the operation.

65 2. The process of claim 1 wherein the chlorite concentration of the liquor is maintained within the range of 0.01% to 2%, based on the weight of available chlorine.

70 3. The process of claim 1 wherein the chlorite

content of the liquor is maintained within the range of 0.02% to 0.03%, based on the weight of available chlorine.

ARCHIE LOUIS DUBEAU.

**REFERENCES CITED**

The following references are of record in the file of this patent:

8

| UNITED STATES PATENTS |           |               |
|-----------------------|-----------|---------------|
| Number                | Name      | Date          |
| 1,254,727             | Poulson   | Jan. 29, 1918 |
| 2,183,142             | Mackenzie | Dec. 12, 1939 |

5

**FOREIGN PATENTS**

| Number  | Country       | Date         |
|---------|---------------|--------------|
| 549,678 | Great Britain | Dec. 2, 1942 |